

July 4, 1939.

M. E. MACKSOUD

2,164,332

APPARATUS FOR APPLYING MIRROR SURFACES TO THE INTERIOR OF LAMP BULBS

Original Filed Aug. 18, 1937



## UNITED STATES PATENT OFFICE

2,164,332

## APPARATUS FOR APPLYING MIRROR SURFACES TO THE INTERIOR OF LAMP BULBS

Michel E. Macksoud, Gloucester, Mass., assignor to Birdseye Electric Company, a corporation of Delaware

Original application August 18, 1937, Serial No. 159,665. Divided and this application November 18, 1937, Serial No. 175,184

11 Claims. (Cl. 91—12.2)

This invention relates to improvements in methods and apparatus by means of which metallic mirror surfaces may be applied to glass surfaces and particularly to the interior surfaces of lamp bulbs.

An object of this invention is to provide an improved method and simplified apparatus by means of which a thin metallic reflecting film of uniform thickness may be easily and simply applied to the interior of lamp bulbs.

A further object of this invention is to provide a method by which reflecting metallic films may be directly applied to the interior of lamp bulbs to provide a highly reflective mirror surface which requires no buffing or polishing.

A still further object of the invention is to provide an improved method for this purpose by means of which the metal to form the film is vaporized and deposited directly onto the glass surface.

The invention also concerns a novel and ingenious device for limiting the area in which the metal film is deposited, thus obviating the need of further treatment to remove surplus metal and obtain a sharp line of demarcation between the reflecting and the transparent areas. It will be obvious that such a device prevents waste of metal.

A novel cooling system is also employed by which the neck of the glass vessel and the support therefor are protected from the effects of the high temperatures generated in the process.

Briefly speaking, the invention utilizes a high frequency induction coil in which is placed an insulated crucible containing the charge of metal to be vaporized. The high frequency process is to be preferred over the process using resistances for the generation of heat to vaporize the metal.

These and other objects and advantages of the invention will be more readily understood and appreciated from the following description of a preferred embodiment thereof, as illustrated in the accompanying drawing.

This application is a division of my copending application Serial No. 159,665, filed August 18, 1937.

Figure 1 is a view in side elevation partly in perspective with some parts broken away and some parts in cross-section;

Figure 2 is an enlarged view in side elevation of the vaporizing unit;

Figure 3 is a view in perspective of the cooling unit;

Figure 4 is a view in vertical central cross-section through the vaporizing unit;

Figure 5 is a plan view of the vaporizing unit; and

Figure 6 is a cross-section taken on the line 6—6 of Figure 1.

A detailed description of the apparatus will be given first, followed by an explanation of the process and the advantages thereof. It may be noted at the outset that the unit of Figure 1, capable of treating one bulb at a time, may, as will be apparent to those skilled in the art, be incorporated into an automatic machine having a plurality of these units so that the bulbs are delivered thereto at one point ready for treatment and removed therefrom at another point in finished form.

In the unit illustrated there is a suitable base 5 of insulating material, on the upper surface of which is secured a sealing stopper 2 made of rubber or other suitable material. The glass envelope to be treated is shown comprising a bulbous portion 1, a neck portion and a terminal portion at the end of the neck which flares outwardly as shown at 3. The stopper 2 is of correct size and proportions to receive the flared end 3 of the envelope and to form an air-tight seal therewith.

Mounted in the base 5 and extending upwardly through the stopper 2 are a pair of heavy electrodes or metal standards 7—7 which are provided at the upper ends with bores 15 in which are mounted smaller metal electrodes 21. The electrodes 21 are provided with slots 23 and may be locked in adjusted vertical positions by means of the set screws 17. These set screws are preferably recessed into the electrodes 7 as shown at 19. Current conducting leads 9 are removably secured to the connectors 11 which in turn are attached to the electrodes 7 by means of the screws 13. The leads 9 which are suitably insulated as illustrated extend to any suitable form of high frequency current source. At 20 are a pair of discs of mica, alundum, or other suitable electrical and heat insulating material. The lower disc 20 through which the electrodes 21 project rests on top of the electrodes 7. The upper disc 20 through which the electrodes 21 project frictionally engages them so that it may be positioned vertically as desired. Its purpose will be described later. The disc 24 through which the electrodes 7 project rests upon the stopper 2 and protects it against charring under the heat developed in the process.

In the upper ends of the electrodes 21 are drilled the holes 25 to receive the arms of legs 29 of the vaporizing unit. The unit is held in place by means of the set screws 27. The form

of vaporizing unit which is generally illustrated at 31 is shown as comprising a small coil of closely wrapped turns 33, the terminal ends of which form legs 29. The material of this coil 5 may be of any metal having a sufficiently high melting point to prevent its deterioration under the heat generated in the process. For example, the coil may be made of tungsten or molybdenum wire or alloys thereof. Other materials are 10 suitable for the purposes, depending upon the particular material to be vaporized to form the film. In addition to the requirement that the melting temperature of the metal of the coil be sufficiently high, it is desirable to use a metal 15 on which there is no dissolving action on the part of the metal vaporized under the temperatures employed. Disposed within the coil is a crucible 35 of material which will not melt, soften or vaporize under the temperatures of the 20 process. Here again molybdenum and tungsten are suitable. In some cases the crucible may be made of carbon, graphite, pure fused magnesia, alumina, or sintered and fused thorium oxide. The crucible is made by boring out or 25 otherwise removing the center of a suitable body of the material to provide the cup or recess 31 in which the material to be vaporized is placed, as indicated at 41 in Figure 4. Interposed between the coil and the crucible is a series of 30 strips 39 of mica which hold the two out of electrical contact (Figure 2). It may be noted that in the temperatures encountered in the process the mica has a tendency to fuse but this is a helpful rather than a harmful occurrence. Of 35 course, other suitable insulating materials may be used for this purpose.

Extending upwardly through the support 5 and the stopper 2 is a tube, the upper end 45 of which opens into the glass envelope and the lower end 40 43 of which provides a means for connection to a suitable vacuum source.

At 53 and 55 are indicated the two sections of a cooling unit which when they hug the neck of the envelope substantially completely encircle 45 it. These sections include substantially semi-circular plates 56 and 60 (Figure 3) of a suitable metal such as copper, to the outer surface of which are secured the flat tubes 52 and 54. The tube 52 is provided with a suitable cooling 50 medium supply pipe 75 which is attached thereto by a fitting 77 and the exhaust connection 79 which is connected thereto by the fitting 81. In a similar way the coil 54 is provided with the cooling medium supply pipe 83 attached thereto by the fitting 85 and the exhaust pipe 87 attached thereto by the fitting 89. The coils are shown in the form of flat thin-walled tubes which closely hug the outer faces of the plates 56 and 60, and the adjacent convolutions are 55 preferably spaced as indicated at 56 to permit circulation of air between them.

Secured to each section near the bottom is a bracket 59 which is pivotally mounted on the support 5 by means of the pivot pins 63. Se- 60 cured to the arms 59 are the arms 61 which are engaged at the lower ends by the springs 73 which lie in the recesses 71 in the support 5. The lower ends of the arms 61 are notched at 65 to receive the ends 69 of the flat springs 67 secured to the support 5. When the cooling sections 53 and 55 are swung outwardly to the dotted position shown at 51 on the right of Figure 1, the springs 67 engage the arms 61 to hold the sections outspread.

76 To heat the glass vessel to annealing tempera-

ture a conventional oven 99 is employed. This oven 99 is well known in the art and forms no part of the invention.

The process in which this apparatus is em- 5 ployed will now be described.

An envelope such as an electric lamp bulb is first cleaned on the inside so as to remove all foreign matter of any kind whatsoever and particularly to remove any grease film that may be on it. It is highly important that any film 10 such as a fatty acid film that may be on the surface be removed. If the surface is not thoroughly clean the hot metallic vapor depositing thereon may react with the greasy film to form blisters, holes, pimples, or other irregularities in 15 the mirror surface with the undesired effect of increasing the tendency of the film to peel off. Any reaction that may occur between the hot metallic vapor and the foreign material present will tend to fog the coating or give it an uneven 20 appearance. One method of cleaning the bulb is to wash the interior with a detergent such as "Alphasol". This is then rinsed out and the surface washed with potassium hydroxide which is also washed out. The interior is then washed 25 with nitric acid and again rinsed, preferably with distilled water. This order of application of the cleaning agents is the reverse of that used in silvering mirrors because fatty acids adhere to the alkaline glass surface more readily than 30 to the acidified glass surface. The bulbs are then dried by placing them neck down in an oven to increase the speed of drying or merely allowing them to dry by exposure to air at ordinary temperatures. The surface to be coated 35 should be so clean, as it will be by this washing method, that when the breath is blown on it a uniform structureless gray film of moisture will form with no apparent pattern. If a pattern in the moisture film is present, this indicates that the surface is not thoroughly clean and should be recleaned. However, if the above 40 cleaning method is carefully followed the surface will be suitably cleaned for the purposes hereof.

It may be noted that "Alphasol" is one of a class of detergents which are sulphonated organic compounds of high molecular weight. They have a neutral reaction and their advantage over soap lies in the fact that they may 45 be used in neutral, alkaline, or acid solutions. Unlike soaps they form soluble compounds with the magnesium and calcium solids common in tap water and therefore rinse easily.

A glow discharge may be employed to finally 50 clean the glass bulb after a vacuum has been produced in it, and while it is mounted on the unit, by applying a high frequency current discharge to one of the electrodes.

Another suitable method of washing and cleaning the bulbs is to wash them with agitation in ammonium bifluoride. The bulbs are then rinsed with water and this may be tap water under pressure and rinsed again with hot or boiling water. Just prior to silvering they are again 55 washed in a bath of stannous chloride followed by thorough washing with distilled water and drying.

They may be cleaned also by washing, using a solution of chromic acid which is prepared by 60 mixing 100 cc. of sulphuric acid with about 4 grams of sodium dichromate. They are then washed out, first with tap water and then with distilled water, and dried.

When thoroughly dried the bulb is placed on 75

the stopper 2 and with the vacuum pump connected to the tube running it is drawn tightly thereon to form an air-tight seal. A fairly high vacuum is desirable and this can be secured by 5 using condensation or diffusion pumps cooled by a dry ice trap in combination with the usual mechanical oil pump. Adequate vacuumizing capacity is desirable, not so much to maintain an extremely high vacuum within the bulb 10 since the degree of vacuum is not critical, but to aid in maintaining a substantial vacuum during the vaporization of the mirror metal. At the beginning of the heating of the crucible and mirror metal there is a substantial "outgassing" and 15 it is desirable that the freed gases be quickly removed from the bulb.

Prior to the application of the bulb to the stopper a suitable quantity of the mirror metal 20 41 is placed in the crucible. A pellet of pure silver is highly satisfactory for the purpose. However, other metals may be employed, such as aluminum, magnesium, chromium, and alloys thereof.

After a vacuum has been created in the bulb 25 and prior to the vaporization of the mirror metal, it is highly desirable that the glass bulb be heated sufficiently high to "de-gas" it. It has been found that if the bulb is heated to the proper degree prior to the vaporization of the mirror 30 metal and maintained substantially at that temperature during the vaporization of the metal, the resulting mirror is deposited with a high lustre and polish equal to the polish of the glass bulb surface and needs no further polishing, 35 buffing or burnishing. The bulbs should be heated to temperatures at least equal to the annealing temperatures of the glass of which they are made. This drives out substantially all occluded gases and removes considerable moisture and residual impurities from the glass. By maintaining 40 the bulb at or near the annealing temperature of the glass during the vaporization process, the glass is kept dry and any further gases which evolve are removed. The result of this treatment is that the resulting metal coating firmly 45 adheres to the glass with little danger of it later peeling therefrom. In addition, this heating contributes to the high lustre and polish of the metal film because the crystalline structure of the deposited film is kept fine. It is important to note 50 that since the annealing temperatures of different glasses vary it is essential that the glass manufacturers' annealing temperatures be followed in the heating of the bulbs.

55 The high frequency current is then supplied to the coil 33 which very rapidly heats the mirror metal to the point of vaporization. It is heated until it has a vapor pressure of the order of one-tenth of a millimeter of mercury. The 60 vacuum is sufficiently high to give a long means free path so that the molecules of the metal travel with substantially no inter-molecular collisions from the crucible to the wall of the envelope. It may be here noted that silver is particularly desirable because of its tendency to 65 clean up any released vapor. That is its "getter" action. Aluminum also displays this characteristic to a high degree. The mirror metal reaches the vaporization point very rapidly and the vapor 70 quickly travels to and condenses upon the inner wall of the envelope to form a thin, clear, uniform film thereon. In accordance with this process and particularly when silver is used, the resulting mirror surface is extremely smooth and 75 highly polished so as to require no further buffing

or polishing operation. The film has no blush and is uniformly clear without pattern or blemish.

The coil 33 and crucible 35, of course, become so hot during the vaporizing step that any mirror metal that deposits on them is immediately 5 vaporized, insuring that the diameter of the wire in the coil 33 does not build up and short circuit the turns and further insuring that the wall thickness of the crucible 35 does not increase.

The upper disc 20 is positioned on the electrode 10 21 at the point at which it is desired to terminate the film. If the disc fits snugly in the neck of the glass bulb the cut-off is sharp, requiring no additional treatment.

During the operation the cooling coils are in 15 the position shown in Figure 1 and any suitable cooling fluid such as air, water, or refrigerating liquid is caused to flow therethrough, protecting the apparatus and particularly the stopper against destruction. The cooling coil also keeps 20 the electrodes and the glass vessel from getting excessively hot during processing. It is important to note that the effectiveness of this process is increased by a rapid condensation of the metal vapor on the glass vessel. For this reason it is, 25 of course, desirable to keep the apparatus itself as cool as possible.

The entire coating has been indicated generally at 49 and is shown more specifically at 47. The reference numeral 22 indicates the line of 30 cut-off of the coating at the edge of the upper disc 20. The region indicated at 51 is a desirable position for the vaporizing unit to insure direct exposure of the inner walls to the vaporized metal and a quick deposit thereof on them. However, 35 the high frequency coil and crucible may be moved to any preferred suitable position to produce the required deposit of the mirror metal vaporized therefrom in any preferred portion of the glass bulb envelope.

40 The vapor condenses quickly and the cooling coil sections are swung outwardly so that the bulb may be removed from the stopper. The dash line 91 indicates the substantial meridian of the bulbous portion and represents the line of cut-off in forming either a directly reflecting bulb or an indirectly reflecting bulb. If a directly reflecting bulb is desired a suitable acid solution such as a nitric acid solution is placed in the bulb while it is held vertical until its level is 45 about at the line 91. This removes the deposit over the area 93 and the acid solution is then removed with a suitable tube. If an indirectly reflecting bulb is desired it is dipped neck down vertically into a bath of nitric acid until submerged to the line 91. This removes the film indicated by reference numeral 95, leaving only the end coated. The line of cut-off is sharp and requires no further treatment. After such acid 50 solution treatment and metallic film removal, the 55 bulb is washed in an ammonium hydroxide solution to counteract the effects of the acid solution and then rinsed in distilled water.

The thickness of the metal film deposited on the glass may, of course, be controlled by varying the amount of metal placed in the crucible. In some cases it may be desirable to build up the film by the application of successive layers which may easily be done by repeating the vaporization step. In some cases it has been found desirable to apply several layers each of a different metal. For example, because of the fact that chromium adheres closely to the glass, even if it has not been thoroughly cleaned, it is sometimes desirable to first deposit a film of chromium 70 75

followed by the deposit thereon of a film of silver or aluminum.

In some cases it may be desirable to apply a protecting coating over the metal film which may be done, for example, by placing a small quantity of quartz in the crucible and vaporizing it so that it is deposited on the metal film. This protects the film against scratching, tarnishing, or other damage without seriously interfering with its light reflecting properties.

10 For ordinary light reflecting purposes, it is desirable to keep the metal film as thin as possible because a higher lustre and polish results. This arises from the fact that in thicker coatings the 15 crystalline structure becomes coarser forming a duller and less reflective film. A film that is just opaque to sunlight seems most efficient as a reflector. Such a film has a thickness of the order 1000 Å.

20 Those skilled in the art will readily appreciate that the details of the apparatus disclosed and the method of procedure may be readily varied without departure from the novel and true scope of this invention. I do not, therefore, desire to be strictly limited to the disclosure as given for 25 the purposes of illustration, but rather to the scope of the appended claims.

What I seek to secure by United States Letters Patent is:

30 1. An apparatus as described comprising a support adapted to receive the neck of a glass vessel and form an air-tight seal therewith, means extending through the support for withdrawing the air from the vessel, a crucible within the 35 vessel, and a heating coil surrounding the crucible and supporting it.

40 2. An apparatus as described comprising a support adapted to receive the neck of a glass vessel and form an air-tight seal therewith, means extending through the support for withdrawing the air from the vessel, a crucible mounted on the support within the vessel, a heating coil surrounding the crucible, and cooling means positioned around the neck of the vessel.

45 3. An apparatus as described comprising a support adapted to receive a glass bulb and form a seal therewith, a tube extending through the support by means of which air may be withdrawn from the bulb when mounted thereon, a pair of electrodes mounted on the support within the bulb, a heating coil connected to the electrodes, a crucible surrounded by the heating coil, and cooling means positioned to surround the neck of the bulb.

55 4. An apparatus as described comprising a support adapted to receive a glass bulb and form a seal therewith, a tube extending through the support by means of which air may be withdrawn from the bulb when mounted thereon, a pair of electrodes mounted on the support within the bulb, an oven for heating the bulb, a heating coil connected to the electrodes, and cooling means positioned to surround the neck of the bulb, said cooling means including a pair of transversely 60 curved members through which a cooling fluid may be circulated.

70 5. Apparatus as described comprising a base of insulating material, means on said base for tightly sealing a glass vessel, a tube extending through said base and within said glass vessel, a pair of electrodes vertically mounted on said base and extending within said vessel, an induction coil carried on said electrodes, a crucible disposed within the convolutions of said coil, a disc of insulating material surrounding said tube and

shielding said base from the interior of said vessel, another insulating disc surrounding said electrodes and fitted to the walls of said vessel, and a cooling system surrounding the upper portion of said base and the neck of said vessel, said cooling system including a pair of concave flattened coils pivotally mounted on said base, whereby said coils may be swung away from said base and said vessel.

6. Cooling system for high frequency metal 10 vaporizing apparatus used to deposit a reflecting film of metal on the interior surface of a glass vessel, which comprises a jacket formed by two semi-circular coils, each coil having an inlet and an outlet for the cooling medium, and a convoluted flat tube connected to said inlet and outlet, and means for pivotally supporting said coils in opposed relation.

7. Apparatus as described comprising a base of insulating material, means on said base for sealing a glass bulb thereto, a tube extending through said base and within said glass bulb, a pair of electrodes mounted in said base and extending within said vessel, an induction coil carried on said electrodes, a crucible disposed within the convolutions of said coil, a first disc of insulating material disposed in said bulb to shield said base from the interior of the bulb, and a second disc of insulating material disposed above said first disc and fitted to the inner surface of said bulb 30 to prevent deposition of metal below said second disc.

8. An apparatus as described including a supporting base having means thereon adapted to support and seal a vessel, said base having a 35 passage open to the space enclosed by the vessel when applied to said means, a pair of vertically adjustable conducting supports mounted on said means so as to be within the vessel when applied, a heating coil attached between said supports, 40 and a crucible mounted within the heating coil.

9. An apparatus as described including a supporting base having means thereon adapted to support and seal a vessel, tubular means extending through the support so as to be open to the space enclosed by the vessel when applied to said means, a pair of vertically adjustable conducting supports mounted on said means so as to be within the vessel when applied, a heating coil attached between said supports, and cooling 50 members movably mounted on said support and positioned so as to enclose the adjacent portions of the vessel when applied to said means.

10. An apparatus as described including a supporting base having means thereon adapted to support and seal a vessel, evacuating means extending through the support so as to be open to the space enclosed by the vessel when applied to said means, a pair of vertically adjustable conducting supports mounted on said means so as to be within the vessel when applied, a heating coil attached between said supports, and a shield mounted on said conducting supports for vertical adjustment within the vessel.

11. In an apparatus of the type described the 65 combination comprising a heating coil composed of a plurality of closely arranged turns of conducting material and supporting legs formed by the terminal ends of the conducting material, a highly refractory crucible enclosed by said coils, 70 and insulating means interposed between said crucible and coils, whereby the coil tightly grips the crucible and insulating means to support them by said legs.